

April 18, 1967

L. R. ERWIN ET AL

3,314,815

METHOD OF APPLYING A PROTECTIVE COATING TO A METALLIC STRUCTURE

Original Filed Feb. 21, 1961



FIG. 1



FIG. 2



FIG. 3

INVENTOR.

LEE R. ERWIN  
DOUGLAS W. MC CALLUM  
RALPH H. GIESER

BY

*Kerman Seid*  
ATTORNEY.

# United States Patent Office

3,314,815

Patented Apr. 18, 1967

1

3,314,815

## METHOD OF APPLYING A PROTECTIVE COATING TO A METALLIC STRUCTURE

Lee R. Erwin, Duarte, Douglas W. McCallum, Hacienda Heights, and Ralph H. Gieser, La Habra, Calif., assignors to Carrier Corporation, Syracuse, N.Y., a corporation of Delaware  
Continuation of application Ser. No. 90,844, Feb. 21, 1961. This application Oct. 25, 1963, Ser. No. 319,046  
1 Claim. (Cl. 117—40)

This application is a continuation of our co-pending application Ser. No. 90,844, filed on Feb. 21, 1961 and now abandoned.

This invention relates broadly to the art of providing a surface of a structural unit with a coating of a material to protect the surface. More particularly, this invention relates to a method of applying a coating of porcelain enamel to a structural unit. Still more particularly, this invention relates to a method of applying a coating of porcelain enamel to a structural unit wherein the surface to be coated has, by its design, an irregular configuration.

In the manufacture of domestic hot water heating units it has been long recognized that the surface of the tank assembly employed in the unit be provided with a lining of porcelain enamel in order that the useful life of the tank be prolonged. The porcelain enamel coating applied to the inner surface of the tank forms what is commercially known as a glass-lined hot water heating unit. The porcelain enamel lining serves as a protective coating for the material forming the tank or water accommodating unit. Usually, the tank is composed of either sheet steel or in some cases, cast iron. As such, it is subject to attack by corrosion. The presence of the porcelain enamel coating on the surface of the tank serves to resist corrosion and thus extend the useful life of the tank.

In the construction of the domestic hot water heating units referred to above, certain economies may be effected by welding the central or cylindrical portion of the tank to an upper or head cover under circumstances where the terminal portions of the two parts are overlapped and the weld made on the outside thereof. With such an arrangement, however, there is presented for coating by suitable porcelain enamel applicator means, a surface formed of a number of sections extending at an angle to one another. Such a structural arrangement tends to form pockets or sheltered areas in the surface to be coated. These pockets are difficult to supply with the porcelain enamel during the coating step for the edges and walls which define the pockets tend to protect them from the spray as it is being applied.

The chief object of this invention is the provision of a method of applying porcelain enamel coating to a structural unit wherein the surface to be coated is irregular in configuration.

This and other objects of the invention which will be apparent upon a consideration of the ensuing specification are attained by the use of a method wherein heat is applied to the portion of the structural unit accommodating the surface irregularity prior to and during the time the porcelain enamel is applied in slip form to the surface of the unit.

FIGURE 1 is a view in section showing a tank assembly of the type used in the fabrication of a domestic hot water heating unit and which contains a surface configuration of the kind with which the invention may be used.

FIGURE 2 is an enlarged fragmentary view showing in section the connection between two of the elements illustrated in FIGURE 1.

2

FIGURE 3 is a somewhat schematic view of a structural unit having a coating of porcelain enamel applied with the method forming the subject of this invention.

In a domestic hot water heating unit the water accommodating tank is composed of a cylindrical shell having end covers secured to opposite ends thereof. In the fabrication of such a unit, it is general practice to connect one end cover to the cylindrical shell member and provide the inner surface of the connected parts with at least one coating of porcelain enamel. The final assembly is completed by coating one surface of the other end cover and connecting it to the assembly described. It will be appreciated that the cover members may be provided with flanged openings for accommodating water delivery and water supply lines as well as flue gas exhaust conduit. However, for convenience, such openings have been omitted from the drawing.

In the construction under consideration here, the end cover and cylindrical shell members 10 and 11, are connected by causing terminal portions 12 and 13, respectively, of the two parts to be overlapped and welded as indicated at 14. The inner surface thus presented for coating by porcelain enamel is shown having an irregular configuration comprising the inner surface 16 of the shell, the inner surface 17 of the end cover and the shoulder 18 defined by the thickness of the end cover which is assembled inside the tank after the welding operation referred to above has been completed. Under the circumstances, it will be obvious that it is difficult to maintain on the shoulder 18, with the usual spray equipment employed, a coating of porcelain enamel. It has been found that the porcelain enamel tends to drain or wash off of this area and in effect, leaves bare the portion of the metal forming the inner surface of the unit in the region of the connection between the surfaces 16 and 17.

Automatic conveying equipment is employed for the purpose of transporting the welded parts to a station where the porcelain enamel is applied to the surface of the unit with spraying equipment conventional in the art. The operation of the spraying equipment is timed with the movement of the conveyor so that once the shell is at the station the automatic spraying head moves into the area defined by the interior of the tank and is retracted slowly to its original position. During the retraction of the spray head porcelain enamel in slip form is sprayed onto the interior surface of the tank. The automatic conveying equipment is supplied with means for rotating the tank continually during the period in which the porcelain enamel is sprayed on the inner surface thereof. This equipment is conventional in the art and it is felt that no further explanation is needed.

As is well known to those skilled in the art, the porcelain enamel slip is composed of a mixture of frit and mill additions, together with a vehicle such as water which permits the mixture to be sprayed in the manner described. The frit and mill additions have been ground to a fineness compatible with the operation of the spraying equipment.

The invention herein contemplated involves supplying heat to that portion of the welded unit wherein the unevenness in the surface configuration exists prior to and during the period in which the porcelain enamel slip is applied to the surface thereof. To this end, a burner is mounted in spaced relation to the conveyor so that it may heat the portion of the structural unit wherein the connection between the head and shell members is located. The operation of the burner is such that upon arrival of the unit at the spraying station the burner is energized and heat is applied immediately to the region referred to above. The supply of heat is continued during

the period in which the spray head extends into and is retracted from the interior of the shell and cover assembly.

By preheating the region of the tank parts in the manner described, a portion of the surface having a temperature in excess of the remainder of the unit is provided. Once the porcelain enamel slip is sprayed onto that region, vaporization of the vehicle occurs such as will decrease the viscosity of the slip and make it less prone to flow away from the area defined by the surface 18 and the adjoining portions of the surfaces 16 and 17. Once the heat is continued, the porcelain enamel slip is further dried and partially sets so that if it is desired to add a second coating to the first coat prior to firing the porcelain enamel, the spraying action of the second coat will not cause the portions of the first coat in the vicinity of the connection to be pitted or washed away.

While the degree of heat does not appear to be critical it is recommended that the temperature be maintained short of causing the moisture in the porcelain enamel slip to boil, which, of course, would cause the porcelain enamel to tend to separate from the surface. On the other hand, the temperature should be high enough so that there is a tendency for the water in the porcelain enamel slip to vaporize and cause the resulting mixture to be more viscous.

While we have described and illustrated a preferred

embodiment of our invention, it will be understood our invention is not limited thereto since it may be otherwise embodied within the scope of the following claim.

We claim:

5 In a method of applying a coating of porcelain enamel to a surface of a structural unit wherein said surface includes angularly related portions presenting an irregular configuration, which comprises the steps of preheating the outer surface of the structural unit in the region of said irregular configuration prior to the application of a porcelain enamel slip to the inner surface of said region, and continuing to heat said unit in the region of said irregular configuration while applying a coating of porcelain enamel in slip form so that the vehicle content of said slip is partially evaporated thus providing a coating of relatively dry porcelain enamel on said inner surface of said structural unit in the region of said irregular configuration.

References Cited by the Examiner

UNITED STATES PATENTS

2,959,851 11/1960 Deringer ----- 29-460

ALFRED L. LEAVITT, Primary Examiner.

RICHARD D. NEVIUS, Examiner.

W. L. JARVIS, Assistant Examiner.